

# United States Patent [19]

Stacey

[11] 3,844,848

[45] Oct. 29, 1974

[54] **PRODUCTION OF LOW ALLOY STEEL WIRE**

[75] Inventor: **Andrew Gordon Stacey**, Norton, near Doncaster, England

[73] Assignee: **British Ropes Limited**, Doncaster, England

[22] Filed: **Nov. 15, 1973**

[21] Appl. No.: **416,203**

[30] **Foreign Application Priority Data**

Nov. 15, 1972 Great Britain ..... 52805/72

[52] U.S. Cl. ..... 148/12 B, 148/12.4

[51] Int. Cl. ..... C21d 9/52

[58] **Field of Search** ..... 148/12 B, 12.4

[56] **References Cited**

UNITED STATES PATENTS

2,756,169 7/1956 Corson et al. ..... 148/12.4

|           |         |                     |          |
|-----------|---------|---------------------|----------|
| 3,011,928 | 12/1961 | Kopec et al. ....   | 148/156  |
| 3,574,000 | 4/1971  | Geipel et al. ....  | 148/12 B |
| 3,584,494 | 6/1971  | Giepel et al. ....  | 148/12 B |
| 3,645,805 | 2/1972  | Hoffman et al. .... | 148/12.4 |
| 3,711,338 | 1/1973  | Vitelli ....        | 148/12.4 |

*Primary Examiner—W. Stallard  
Attorney, Agent, or Firm—Johnson, Dienner, Emrich,  
Verbeck & Wagner*

[57]

## ABSTRACT

Low alloy steel rod is given a pearlite structure and is then cold-drawn to initiate work hardening. The rod is then drawn through a die producing a reduction in area of between 10 and 40 percent. The wire leaving the die is heated to 300°-450°C and then forcibly cooled.

**5 Claims, No Drawings**

## PRODUCTION OF LOW ALLOY STEEL WIRE

The present invention relates to low alloy steel wire.

The mechanical properties of drawn carbon-steel wire can be manipulated and controlled by subjecting the wire to oil quench hardening and tempering. It would be desirable to be able to treat low alloy steel so as to produce wire which has better mechanical properties than oil quench hardened and tempered wire, especially lower relaxation.

Great Britain Pat. No. 748,357 describes a method of treating cold drawn wire, in which the wire is drawn to its final size in a die and, as it leaves the die, is heated to a given temperature and then quenched, while it is subjected to a tensile stress sufficient to induce permanent elongation. According to Great Britain Patent No. 889,588, the wire may be heat treated, before the final drawing operation, by heating the wire to above the  $AC_3$  point followed by isothermal quenching to about 375°C.

Great Britain Patent No. 1 285 998 describes a method of making low-alloy steel wire, in which wire

(preferably 28 percent); heating the wire leaving the die to 300°-450°C (preferably 420°C); and forcibly cooling the wire.

It can be seen that the reduction in area is low (10-40 percent); the tension on the wire leaving the die is only that needed to draw it through the die and does not necessarily produce permanent elongation; and the temperature to which the wire is heated is quite low (300°-450°C).

The heat treatment to produce the pearlite structure preferably comprises heating above the  $AC_3$  point, cooling to and holding at a temperature between 550° and 700°C, the preferred temperature being 650°C, followed by cooling in air. Of course, the heat treated rod will be cleaned and given a drawing coat before the initial drawing pass.

The invention will be described further, by way of example only, with reference to three steel compositions, viz. a carbon steel: 0.67 percent Swedish carbon steel; and two low alloy steels: British Standard EN 47 (chromium-vanadium) and EN 48a (silicon - chromium). The analyses of the three steels are shown in Table I.

TABLE I

| Specification, wt% | C         | Mn        | S        | P        | Cr        | V       | Si        |
|--------------------|-----------|-----------|----------|----------|-----------|---------|-----------|
| Swedish            | 0.65-0.80 | 0.40-0.80 | 0.040max | 0.040max | —         | —       | 0.35max   |
| EN 47              | 0.45-0.55 | 0.50-0.80 | 0.050max | 0.050max | 0.50-0.80 | 0.15min | 0.50max   |
| EN 48a             | 0.50-0.60 | 0.60-0.90 | 0.050max | 0.050max | 0.55-0.85 | —       | 1.35-1.65 |

material is first given a heat treatment involving heating to a temperature 50°-150°C above the  $AC_3$  point, air cooling to just above the  $Ms$  point, and reheating to 450°-650°C, followed by air cooling. Then follows multi-hole cold drawing to the finished size, with a reduction in area of at least 40 percent. The finished wire is tempered, preferably at 440°C or higher, without tensile stress or quenching. The steel has a high silicon content.

Neither of these methods is applicable to a wide range of low alloy steels.

The present invention provides a method of producing low alloy steel wire from low alloy steel rod, the method comprising heat treating the rod to produce a pearlite structure; cold drawing the rod to initiate work hardening and thereby raise the tensile strength; drawing the part-drawn rod through a drawing die to reduce the cross-sectional area by between 10 and 40 percent

35 "As-rolled" rod (5 mm diameter) of each steel composition was initially austenitised, cooled to 650°C and held at this temperature, and then allowed to cool in air; this provided a pearlite structure. The rod was cleaned, provided with a drawing coat, and drawn to a diameter of 4.4 mm; this initiated work hardening and raised the tensile strength.

40 The part-drawn rod was then further drawn, during which operation it was subjected to a reduction in area of 25 percent, to finish at 3.85 mm diameter. As soon as the wire emerged from the die, it was heated to 420°C and then quenched from this temperature by forcible cooling using an air blast or water spray.

45 The resulting wire had a tensile strength ranging from 158 to 175 kgf/mm<sup>2</sup>. The mechanical properties of the wire obtained from each steel composition are shown in Table II. The properties of the as drawn wire (not heated after drawing) are shown for comparison.

TABLE II

| WIRE                                 | Cr-V  | Cr-V as drawn | Si-Cr | Si-Cr as drawn | 0.69% C. | 0.69% C as drawn |
|--------------------------------------|-------|---------------|-------|----------------|----------|------------------|
| Size : mm,                           | 3.86  | 3.85          | 3.86  | 3.85           | 3.83     | 3                |
| UTS <sup>2</sup> kgf/mm <sup>2</sup> | 175.2 | 171.8         | 166.0 | 158.9          | 170.0    | 176.5            |
| (0.2                                 | 172.6 | 151.2         | 160.9 | 136.6          | 148.2    | 146.5            |
| % P.S. (0.1                          | 171.5 | 138.7         | 158.5 | 123.3          | 146.2    | 128.8            |
| (0.01                                | 153.3 | 88.0          | 134.5 | 70.9           | 130.2    | 77.3             |
| L of P kgf/mm <sup>2</sup>           | 132.5 | 68.7          | 106.8 | 53.7           | 112.8    | 58.0             |
| % P.S. (0.2                          | 98.5  | 88            | 96.8  | 85.9           | 87.0     | 82.7             |
| as (0.1                              |       |               |       |                |          |                  |
| % UTS (0.01                          | 87.6  | 51.2          | 81.0  | 44.6           | 76.4     | 43.8             |
| L of P (% UTS)                       | 75.5  | 40.0          | 64.3  | 33.8           | 65.8     | 32.8             |
| Ex10 <sup>-3</sup>                   | 21.1  | 19.6          | 20.3  | 18.7           | 21.2     | 19.3             |
| % El. 50mm.                          | 9.0   | 5.0           | 9.0   | 6.0            | 8.5      | 4.0              |
| % El. 250mm.                         | 4.2   | 2.0           | 5.2   | 2.6            | 5.0      | 1.4              |
| 5 R of A                             | 54.   | 55            | 56    | 58             | 49       | 53               |
| Torsion on 100x dia.                 | 22    | 28            | 27    | 42             | 25       | 33               |

TABLE II—Continued

| WIRE                                        | Cr-V   | Cr-V as drawn | Si-Cr   | Si-Cr as drawn | 0.69% C. | 0.69% C as drawn |
|---------------------------------------------|--------|---------------|---------|----------------|----------|------------------|
| Torsion quality<br>Bends on 10mm<br>radius. | A<br>8 | A<br>10       | A<br>13 | A<br>14        | A<br>6   | A<br>9           |

UTS=ultimate tensile strength

L of P=limit of proportionality

R of A=reduction of area at fracture

P.S.=proof stress

E=Young's modulus

Wire from all three steels shows a remarkable increase in flow stress characteristics after the heat-treatment at 420°C followed by quenching; the 0.2 percent proof stresses are superior to those normally achieved by oil hardening and tempering.

The results obtained for the low alloy steels are significantly better than those for the carbon steel. A possible explanation is that low temperature heat treatment under tension may promote a dislocation locking mechanism involving interstitial carbon and nitrogen atoms, creating a condition similar to strain ageing. Additions of such alloying elements as chromium, silicon, and vanadium, may promote an interaction between dislocations and alloy carbides, resulting in a further increase in flow stress.

Alloying elements which appear to have an influence on flow stress are listed in Table III together with the percentage ranges within which the influence appears to be significant.

Various modifications may be made within the scope of the invention. For instance, the rod can be given the pearlite structure by a heat treatment comprising controlled cooling of the rod as it leaves the hot rolling mill.

TABLE III

| Element    | Weight%    |
|------------|------------|
| Carbon     | 0.30/1.00  |
| Manganese  | 0.20/1.50  |
| Silicon    | 0.10/4.00  |
| Chromium   | 0.10/4.00  |
| Sulphur    | 0.00/0.050 |
| Phosphorus | 0.00/0.050 |
| Molybdenum | 0.10/2.00  |
| Copper     | 0.10/3.00  |
| Nickel     | 0.10/5.00  |
| Titanium   | 0.10/2.00  |

TABLE III—Continued

| Element  | Weight%   |
|----------|-----------|
| Vanadium | 0.00/2.00 |
| Nitrogen | 0.00/0.50 |
| Niobium  | 0.10/3.00 |

I claim:

1. A method of producing low alloy steel wire from low alloy steel rod, the method comprising heat treating the rod to produce a pearlite structure; cold drawing the rod to initiate work hardening and thereby raise the tensile strength; drawing the part-drawn rod through a drawing die to reduce the cross-sectional area by between 10 and 40 percent; heating the wire leaving the die to 300°-450°C; and forcibly cooling the wire.

2. A method as claimed in claim 1, in which the heat treatment to produce a pearlite structure comprises heating above the  $AC_3$  point, cooling to and holding at a temperature between 550° and 700°C, and then cooling in air.

3. A method as claimed in claim 2, in which the holding temperature between 500° and 700°C is 650°C.

4. A method as claimed in claim 1, in which the heat treatment to produce a pearlite structure is carried out on rod leaving a rolling mill.

5. A method as claimed in claim 1, in which the low alloy steel of which the rod is made contains, by weight: C 0.30-1.00 percent, and alloying elements selected from the following elements in the following ranges: Mn 0.20-1.50%, Si 0.10-4.00%, Cr 0.10-4.00%, S 0.050% maximum, P 0.050% maximum, Mo 0.10-2.00%, Cu 0.10-3.00%, Ni 0.10-5.00%, Ti 0.10-2.00, V 2.00% maximum, N 0.50% maximum, and Nb 0.10-3.00%, the balance being Fe and impurities.

\* \* \* \* \*